

KIYONAO ISHIDA, OF TOKYO-FU, JAPAN.

## PRINTING INK.

1,410,572.

Specification of Letters Patent. Patented Mar. 28, 1922.

No Drawing.

Application filed July 20, 1921. Serial No. 486,183.

*To all whom it may concern:*

Be it known that I, KIYONAO ISHIDA, a subject of the Emperor of Japan, residing at No. 2 of 135 Oaza-kamishibuya, Shibuya-machi, Toyotama - gun, Tokyo - fu, Japan, have invented new and useful Improvements in Printing Ink, of which the following is a specification.

This invention relates to a method of 10 manufacturing a printing ink by mixing together lamp black, mineral oil, rosin, catechu, formaldehyde, alkaline silicate, alkaline carbonate, gum arabic, insoluble soap, and water, the object being to supply a 15 printing ink never smearing papers, nor affecting rolls, so as to secure clear print, its thickness being made adjustable by water admixture.

Among the important qualities a printing 20 ink should have, are counted suitable adhesive power and consistency. If too adhesive, the ink tends to conglomerate and does not spread evenly over the surfaces of rolls, types, or papers, causing thereby 25 various hitches in the printing process. If not sufficiently adhesive, the ink is liable to be pressed from between types and papers, thereby smearing the print. If too consistent or tough, the ink is not easily absorbed by papers so that the printing speed 30 has to be reduced in order to get clear print. If not sufficiently consistent, however, it will penetrate too deeply into the tissue of the paper and smear it.

35 The present invention intends to be a new improvement in these respects. The adhesive power as well as the consistency is so made as to be regulated by adding suitable quantity of water according to changes of 40 atmospheric temperatures or qualities of papers used, while the ink is so prepared as not to affect rolls.

A practical numerical example of the present method is given below:

|    |                                               |                   |
|----|-----------------------------------------------|-------------------|
| 45 | Lamp black                                    | 100 lb.           |
|    | Mineral oil                                   | 1000-2000         |
|    | Rosin                                         | 50-200            |
|    | Catechu                                       | 5-10              |
| 50 | Formalin                                      | 2-10              |
|    | Sodium silicate                               | 10-100            |
|    | Sodium carbonate                              | 2-5               |
|    | Gum arabic                                    | suitable quantity |
| 55 | Aluminium resinate or<br>other aluminium soap | small quantity    |
|    | Colouring matter                              | small quantity    |
|    | Water                                         | 500-2000          |

To combine these ingredients, we first mix rosin with mineral oil; boil the mixture, adding later lamp black. Knead the same 60 with rolls several times, and then add thereto another mixture composed of the rest of the ingredients. Thus the ink is obtained.

Colouring matter here to be used serves to give glossy lustre to the black ink, the 65 black colour being produced from lamp black. For coloured inks, other than black, lamp black is dispensed with, and colouring matter alone is used to produce the required colour. The chief colouring matter 70 used for these purposes are Prussian blue and methyl violet, etc.

Sodium silicate serves to make the ink easy to spread, and besides, in conjunction with gum arabic, it serves to keep oleic ingredients and water fused together in state of emulsion.

Aluminium soap supplies cohesive power to mineral oil, and keeps that power from changing according to atmospheric temperature, it also gives lustre and water-repelling power to the printed surface.

Rosin increases the cohesive power of mineral oil and also supplies consistency.

Catechu tends to prevent smearing and 85 increases lustre of the printed surface and enables the surface to stand friction.

To formalin we owe the durability of glutinous rolls.

These ingredients, however, may be substituted by other similarly acting substances.

Thus it will be seen that the present method is characterized by supplying tannin, soluble silicate, insoluble soap, formaldehyde, and gum arabic to the soap composed of lamp black, mineral oil, resin, etc., thereby enabling the ink to combine and mix with water with the result that the adhesive-ness or viscosity of the ink can be regulated by adding water, which is a great merit. 100 Thus the ink can spread itself easily over surfaces; is equally adhesive; never smears papers; glossy black (or other coloured) with small quantity; the printed surface clear; figures or scenery as vivid as if in 105 relief; never wearies the eyes; the type surfaces and papers easily separable and so that printing speed is gained.

## Claims:

1. A printing ink composed of colouring 110 matter, mineral oil, resin, soluble silicate, water-insoluble soap, a material containing tannic acid, gum arabic and formaldehyde.

2. A printing ink composed of colouring

matter, mineral oil, resin, soluble silicate, water-insoluble soap, catechu, gum arabic and formaldehyde.

3. A printing ink comprising mineral oil, 5 resin, catechu, formaldehyde, sodium silicate, alkaline carbonate, gum arabic, alu-

minium soap, colouring matter and water, substantially as and for the purposes hereinbefore set forth.

In testimony whereof I have signed my 10 name to this specification.

KIYONAO ISHIDA.